

Sept. 20, 1938.

J. FLETCHER

2,130,530

COATING OF FIBROUS SURFACES

Filed Oct. 5, 1935



INVENTOR.

*John Fletcher*  
By

Parker, Prochnow & Farmer  
ATTORNEYS.

## UNITED STATES PATENT OFFICE

2,130,530

## COATING OF FIBROUS SURFACES

John Fletcher, Kenmore, N. Y., assignor to Plasteron Wall Board Company, Buffalo, N. Y., a corporation of New York

Application October 5, 1935, Serial No. 43,738

11 Claims. (Cl. 91—70)

This invention relates to the coating of fibrous surfaces or paper sheets, and particularly to the coating of the paper web leaving a paper making machine.

5 An object of the invention is to provide an improved method of applying a coating to a fibrous surface or sheet, with which the penetration of the coating material into said surface or sheet will be relatively slight, with which a fibrous surface 10 may be coated in a simple, rapid and inexpensive manner, with a minimum of handling of the object to be coated, and with a minimum of manual labor.

Another object of the invention is to provide 15 an improved method of coating a fibrous sheet, such as paper, with which the coating material will remain largely on the surface of the sheet, with which the finish as to gloss or flatness may be varied within limits, and which may be easily 20 and inexpensively performed.

Another object of the invention is to provide 25 an improved method of coating a travelling paper sheet or web, such as the web leaving the drying rolls or cylinders of a paper making machine, and with which the coating may be applied to the web and hardened in a rapid, simple and inexpensive manner while the web is travelling and then be immediately wound or otherwise disposed of.

30 A further object of the invention is to provide an improved method of coating and coloring a fibrous sheet, such as a paper sheet, with which uniformity in the coating and coloring may be obtained, with which the coating and coloring 35 may be performed while the sheet is travelling, and which requires no complicated or elaborate apparatus.

Another object of the invention is to provide 40 an improved method of coating paper and similar sheets with a water dispersion of coating substances, such as nitro cellulose lacquers, synthetic resins, natural fossil resins and rosin.

Another object of the invention is to provide 45 improved apparatus for applying water dispersions of lacquers, resins, rosins and other coating materials which harden by evaporation of solvents, to fibrous objects, such as paper webs and sheets, and which will be relatively simple, inexpensive, and easily incorporated in the usual 50 paper making machines.

Other objects and advantages will be apparent 55 from the following description of an embodiment of the invention, and the novel features will be particularly pointed out hereinafter in connection with the appended claims.

In the accompanying drawing, I have illustrated diagrammatically an apparatus for applying a water dispersion of coating material to a travelling paper web, as the web leaves the drying cylinders or rolls of a paper making machine 5 in order to illustrate an important embodiment of the invention.

Lacquer emulsions or lacquer dispersions in the water phase, have recently been made available for industrial use as also water dispersions of 10 various other coating materials of the type which harden upon the evaporation of a solvent, among which may be mentioned nitro cellulose lacquers, synthetic resins, natural fossil resins and rosin. A description of lacquer emulsions or water dispersions and their preparation, composition and use has recently been published and made available to the trade by The Hercules Powder Company Inc. of Wilmington, Delaware, in a booklet 15 entitled "Lacquer Emulsions", and copyrighted in 20 1935 by The Hercules Powder Company Inc.

Referring particularly to the drawing, the invention is illustrated as it has been successfully applied to a paper making machine for the coating of the travelling paper web leaving the paper 25 making machine. The travelling web 10 of freshly formed paper, after passing over a desired number of drying cylinders or rolls 11, is conducted over an idler cylinder 12 to the upper end of a calendering device or unit 13. This 30 calendering device includes a series of floating, calendering cylinders 14, 15, 16, 17, 18 and 19 which are arranged above one another, guided for vertical movement in floating contact with one another, and yieldingly urged in contact with 35 one another under heavy pressure. Such a calendering device is a common attachment to or a part of paper making machines for calendering the web leaving the drying cylinders.

The web 10 passes alternately around these 40 calender rolls 14 to 19, and then passes from the lower cylinder or roll 19 to the top cylinder 20 of a second calender device or unit 21. As the web 10 passes around the calender rolls in the unit 13, the opposite faces of the web are successively moistened by water applied to the cylinders or rolls 15 and 18 which engage opposite faces of the web, the application of moisture to these rolls or cylinders being obtained by water boxes 22 and 23, each of which is fitted against 50 a side of a cylinder, with the cylinder forming a side wall of the box, the box running approximately for the full length of the cylinder. This is common practice in the calendering devices of 55 paper making machines.

The second calender unit 21 includes, in addition to the top cylinder 20, additional cylinders 24, 25, 26, 27 and 28 all arranged as usual in paper making machines in superposed, floating contact with one another, and under high pressure on one another. The web 10, after passing over the top calender roll 20, passes alternately around the lower rollers 24 to 28 of that unit, and then passes to the top roller 29 of another 10 calender unit 30. The web, after passing around the top roller 29 of this third unit 30, passes alternately around the successive and lower rolls 31, 32, 33, 34 and 35 of that unit, and then is conducted over an idle roller 36 to the winding 15 or cutting mechanism, as usual in paper making machines. These three units 18, 21 and 30 thus represent three usual calendering units through which the web is commonly passed successively in leaving the drying cylinders before it is wound 20 or otherwise disposed of.

In the unit 21, two of the rollers or cylinders 25 and 26 intermediate the top and bottom rollers are heated in any suitable manner such as by steam, and similar rollers 32, and 33 in the unit 25 30 may also be similarly heated. A water box 37 is disposed along the roller 27 which is below the heated rollers 25 and 26 in the intermediate calender unit 21, so as to apply a liquid coating to the cylinder 27 and through it to one face of the 30 travelling web 10. In this water box 37, of which the cylinder 27 forms one side wall, I place the water dispersion of the coating material, and thus as the cylinder 27 rotates in the direction of the arrow, it will carry some of this coating material with it and transfer it to one face of the 35 travelling web 10.

The water dispersion of the coating material may be prepared in any desired manner and of any desired material, but among such materials 40 which are particularly useful in the coating of paper may be mentioned the nitro cellulose lacquers, synthetic resins, natural fossil resins, rosin, particularly the rosin which is the residue from the distillation of turpentine from turpentine sap, 45 and also oil and water soluble termite and fungus resisting materials, as well as water dispersions of insoluble termite and fungus resisting materials. Fungus and termite resistant materials are well known, and include arsenic compounds, coal 50 tar products and certain zinc salts. Various mixtures of these materials to make up the coating compound, in water dispersion phase, may be used when desired.

The water dispersion or emulsion of the coating material which is placed in the water box 37, 55 may also contain any desired coloring material, either of the water or oil soluble type. The preferred dyes are soluble in coal tar solvents, or in solvents which are immiscible with water, or with 60 pigments in suspension, so as to impart to the coating any desired color.

In the operation of this coating apparatus, the paper web 10 which leaves the drying rolls or cylinders 11 of the paper making machine is of a 65 temperature materially above room temperature, and as it passes through the calendering unit 18, the opposite faces of the web are moistened by water contained in the water boxes 22 and 23. At the same time the web is subjected to considerable pressure as it passes between abutting rollers of the unit 18. In the making of paper, it is necessary to dry the web quite thoroughly throughout, and then to moisten the faces thereof in order to calender the surfaces of the web. 70

75 After being moistened on its faces and sub-

jected to pressure in the unit 18, as usual heretofore, the web passes through the second unit 21 in which the web is subjected to further pressure between the cylinder rolls of that second unit, the web being heated further as it passes 5 around the rollers 25 and 26. The heated web leaving the roller 26 passes in contact with the roller 27, which forms one side of the water box 37 in which the water dispersion of the coating material is placed, and the roller 27 takes up a film 10 of this coating material from the box 37 and carries it into contact with the web 10 on one face thereof, excess coating material of the film being squeezed out by the pressure between the rollers 26 and 27 and running back into the box 37. The 15 coated face of the web then passes between the rollers 27 and 28 where it is subjected to pressure to force the coating compound into further contact with the web fibres, and then this coated face is exposed to air as it passes around the roller 28 20 and travels to the top of the third calender unit 30.

As this freshly coated web leaves the roller 27 and passes in contact with the air to the third calendering unit 30, a considerable portion or all 25 of the volatile solvent of the coating is driven off by evaporation, it being understood that the freshly coated web in this zone has a temperature above room temperature, and the escape of steam and moisture from the web when so exposed to air aids in carrying off the volatile solvent, with the result that by the time the web reaches the top roller of the third calender unit, 30 the coating has set to some extent so that it is no longer tacky. 35

This partially dried or hardened coated web is then passed through the calender unit 30, between the successive rollers thereof, where it is subjected to a calendering operation of pressure and heat, during which any remaining solvent 40 and the moisture in excess of that desired in the finished web is driven off, and a smooth calendering surface is provided on the coated web. The web then passes over the roller 36 to the winding roller or the cutting machine as usual 45 in paper making machines.

In the foregoing description, it will be understood that the coating may be applied through the water box of the usual calendering mechanism of paper making machines, without any increase in equipment or any additional handling of the web, but if it is desired to coat both faces of the web, an additional calendering unit should preferably be provided, so that the opposite faces of the web may be successively coated and then 55 a drying and calendering finish given to the web.

It will be understood that the apparatus illustrated diagrammatically in the drawing, and which constitutes part of a well known paper making machine, may be modified within the principle of this invention, and the improved method of coating may be applied to flat sheets by performing similar operations on the web, such as, for example, by first moistening the face of the web to be coated, then calendering it, applying a 65 water dispersion of the coating material thereto, allowing the volatile solvents and part of the moisture to evaporate, and then further calendering or drying the coated sheet.

I have found that by first moistening the web 70 before the water dispersion of the coating material is applied thereto, there is less penetration of the coating material into the fibers of the sheet, also that the heating of the web or sheet before the water dispersion of the coating 75

material is applied is advantageous, in that the heat of the web quickly eliminates the volatile solvent of the coating material in a steam atmosphere, and also part of the moisture of the coating, so that less travel of the web and less exposure of the web to air is required before being further calendered and dried. The driving off of the solvent in an atmosphere of steam which occurs while the web is travelling between the units 21 and 30 tends to produce a mat finish on the web, which is particularly valuable as a primer coat or finish to receive paints, particularly water paints. If a higher gloss on the coated face of the web is desired, the preliminary moistening of the web before the water dispersion of the coating material is applied is eliminated or the amount of preliminary moistening reduced. The preparation of the water dispersion of various substances is now generally understood and is explained in the booklet entitled "Lacquer Emulsions" hereinbefore referred to. The preparation of such an emulsion may, however, be briefly described as follows:

The first step in preparing a lacquer emulsion is to make up the base lacquer. The composition of this base lacquer depends upon the use to which the finished lacquer emulsion is to be put.

The lacquer base and water containing the emulsifying agent are then mixed together, and agitated to obtain a uniform mixture which can be put through an emulsifying machine such as the Premier Colloid Mill or The Manton-Gaulin Homogenizer. However, many other machines of similar type are available, which probably would give comparable results. The ratio of lacquer phase to water phase will ordinarily vary between 2 parts of lacquer to 1 part of water and 3 parts of lacquer to 1 part of water. In general, the lower the percentage of water used in the emulsion, the higher the viscosity of the finished emulsion will be. In making all emulsions and especially those with a low percentage of water, it is best to use a procedure known as "Seeding". By this procedure about a quarter of the lacquer base is first dispersed in the entire water phase and this mixture is passed through the homogenizer to form a dilute emulsion. To this is then added the remaining three-quarters of the lacquer base and the complete mixture again is emulsified. The size of the emulsion particles is decreased by repeated passes through the homogenizer. One or two passes is usually sufficient however.

In making up a pigmented lacquer emulsion on the Manton-Gaulin, the following technique is recommended. The baffle ring on the second stage homogenizer should be left out and a properly supported 200-mesh screen placed over the outlet of the second stage homogenizer. All of the water phase should be added first with only a small part of the lacquer phase, and pumped through the machine; the only pressure should be that built up by the resistance of the screen. The remainder of the lacquer phase is gradually added during recirculation. When it is all added, the first stage pressure is increased to 2,500 pounds, and 1,500 pounds is put on the second stage. The emulsion is then passed through the machine two or three times. The same technique may be used on the unpigmented emulsions though they are usually made without the screen and with the second stage baffle ring in place.

There is a distinction in the drying of a solu-

tion of nitro cellulose in solvent. Such a solution dries by evaporation of the solvent, depositing a uniform continuous film, and with the addition of resin a glossy film. A flocculation of the solids occurs on the coated sheet or web when a water phase dispersion of nitro cellulose in solvent is used as the coating material. The evaporation of the solvent and the water flocculates the solids and this flocculation deposits on the fibers.

This coating has a mat appearance and is particularly suitable for its intended use as a priming or base coat for finish coats of clear lacquer or nitro cellulose in solvent.

Nitro cellulose dispersion in the water phase has a milky appearance.

It will be understood that various changes in the details, materials and steps which have been herein described and illustrated in order to explain the nature of the invention, may be made by those skilled in the art within the principle and scope of the invention as expressed in the appended claims.

I claim as my invention:

1. The method of coating the fibrous surface of a sheet-like object, which comprises pre-wetting said surface with water, applying to the said wet surface a coating of a water dispersion of a nitrocellulose lacquer containing a solvent for the nitrocellulose, then exposing the coated object to a drying, humid atmosphere sufficient to eliminate the solvent without substantial elimination of the water and deposit the nitrocellulose lacquer solids on said surface, and then drying the object to remove the water.

2. The improved method of applying a coating to a surface of a fibrous object which comprises moistening the surface of the object with water, applying to the moistened surface a coating of a water dispersion of a nitrocellulose lacquer, drying the coated object until the coating passes the tacky stage, and then further drying and calendering the coated surface to produce a mat-like finish on the coating.

3. The improved method of applying a coating to a surface of a fibrous object which comprises moistening the surface of the object with water, heating the object, applying to the moistened and heated surface a coating of a water dispersion of a nitrocellulose lacquer, drying the coated object until the coating passes the tacky stage, and calendering the partially dried, coated surface to produce a mat-like finish on said coating.

4. The improved method of coating a paper web which comprises imparting translation to said web, heating and moistening the face of said web to be coated, applying to the heated and moistened face of the moving web a coating of a water dispersion of a nitrocellulose lacquer, drying the coated web while in motion until the coating passes the tacky stage, and then calendering the coated surface with heat to dry the coated web and produce a mat-like finish on the coating.

5. The improved method of coating a surface of a fibrous object which comprises applying to said surface while in a heated and moist condition, a coating of a water dispersion of a nitrocellulose lacquer, drying the coated surface until the coating passes the tacky stage, and then calendering the coated surface with heat to further dry the coated web and produce a mat-like finish on the coating.

6. The improved method of coating a paper web which comprises applying to the hot, moist

5 web leaving the drying cylinders of a paper making machine, a coating of a water dispersion of a nitrocellulose lacquer containing a volatile solvent for the nitrocellulose, passing the coated web in contact with air to partially eliminate the volatile solvent in said coating and carry the coating on the surface past approximately the tacky stage, and then calendering and further drying the coated web to produce a mat finish  
10 on the web.

7. The improved method of coating a paper web which comprises translating said web while heated and moistened on that surface which is to be coated, applying to the moistened and heated surface a water dispersion of a nitrocellulose lacquer, exposing the travelling coated web to a drying action until the coating passes approximately the tacky stage, and then calendering the travelling coated web with heat to harden and dry the coating and produce a mat-like finish thereon.

8. The method of coating a paper sheet which comprises coating a face of the sheet which, before coating, contains substantially more moisture than it will retain in normal atmospheric conditions, with a water dispersion of a nitro-cellulose lacquer containing some volatile solvent for the nitrocellulose, and immediately exposing the coated sheet to a drying atmosphere at a temperature above normal room temperature to eliminate the solvent and deposit the lacquer solids on said surface, and then eliminating the remaining water from said deposited coating.

9. The improved method of coating a paper web which comprises applying to the traveling, hot, moist web leaving the drying cylinders of a paper making machine, a coating of a water dis-

ersion of a nitrocellulose lacquer and containing intermixed therein a termite and fungus resistant material, said dispersion containing a volatile solvent for the nitrocellulose, then passing the hot coated web immediately in contact with air to partially eliminate the volatile solvent in said coating sufficiently to quickly carry the coating on the surface past approximately the tacky stage, and then further drying the coated web.

10. The improved method of coating a paper web which comprises continuously applying to the traveling, hot, moist web leaving the drying cylinders of a paper making machine, a coating of a water dispersion of a nitrocellulose lacquer containing a volatile solvent for the nitrocellulose, then immediately passing the hot coated web in contact with air to quickly and at least partially eliminate the volatile solvent in said coating sufficiently to carry the coating on the surface past approximately the tacky stage, and then further drying the coated web.

11. The improved method of applying a coating to a surface of a fibrous object which comprises coating a face of said object which before coating contains substantially more moisture than it will retain under normal atmospheric conditions, and while at a temperature substantially above normal room temperature, with a water dispersion of a nitrocellulose lacquer containing some volatile solvent for the nitrocellulose, then immediately exposing the hot coated sheet to contact with air to partially eliminate the volatile solvent in said coating sufficiently to carry it past approximately the tacky stage, and then further drying the coated object. 25 30 35

**JOHN FLETCHER.**